

Aug. 9, 1932.

R. H. HOBROCK

1,871,269

## METHOD OF DRYING MATERIALS

Filed Sept. 25, 1929

Fig. 1.



Fig. 2.



Fig. 3



30 Fig. 5.



Fig. 4.



inventor  
Raymond H. Hobrock  
By Hal Patterson Atty.

## UNITED STATES PATENT OFFICE

RAYMOND H. HOBROCK, OF CHICAGO, ILLINOIS, ASSIGNOR TO WESTERN ELECTRIC COMPANY, INCORPORATED, OF NEW YORK, N. Y., A CORPORATION OF NEW YORK

## METHOD OF DRYING MATERIALS

Application filed September 25, 1929. Serial No. 395,103.

This invention relates to a method of drying materials, and more particularly to a method of drying materials having a normal moisture content.

5 One of the most serious difficulties encountered in the manufacture of certain types of electrical condensers results from the reluctance which small vestiges of moisture, remaining in paper employed as a dielectric 10 in the condensers, exhibit under attempts to remove them.

An object of the invention is to provide a simple method for drying material, and one which will be of uniform and maximum efficiency.

A preferred embodiment of the invention contemplates the application, through the paper dielectric, of a high potential, which due to the pronounced polarity existing in all 20 water molecules and the relation of specific inductive capacity and charge existing between the water and the walls of the capillary openings drives the minute particles of moisture contained in the capillaries of the paper 25 to the surface, whence it is evaporated by heat.

The invention will be more fully understood from the following detailed description, reference being made to the accompanying drawing forming a part thereof, in which

30 Fig. 1 is an enlarged fragmentary transverse sectional view of a condenser, shown composed of wound paper and tin foil, arranged in alternate layers;

35 Fig. 2 is a further enlarged fragmentary section taken on the line 2—2 of Fig. 1, showing the condition of a capillary after an initial heat treatment;

40 Fig. 3 is a view corresponding to Fig. 2, showing the condition of the capillary during a second heat treatment and before a potential is applied across the dielectric;

45 Fig. 4 is a view corresponding to Fig. 3 showing the condition of the capillaries after the potential has been applied; and

Fig. 5 is a diagrammatic view of an electric circuit employed in the process.

50 Referring to the drawing, in which similar parts are indicated by identical reference

numerals, a condenser 10 includes a lead 11 preferably composed of thin sheet metal such as tin, copper or other suitable electrical conducting material. The lead 11 has secured thereto at one end thereof one end of a sheet 55 of tin foil 12, which in turn is engaged by one end of a sheet of paper 14. The condenser 10 also includes a second lead 15, similar to the lead 11, spaced therefrom and having secured to one end thereof one end of a second tin foil sheet 16 which is engaged by one end of a second sheet of paper 17. It will be understood that the sheets of tin foil and paper may be, as in ordinary practice, several feet in length, dependent upon the 60 capacity which it is desired that the condenser possess. In forming the condenser, leads 11 and 15 are held in their spaced relation by any suitable means (not shown), while the tin foil and paper sheets from each 65 of the leads 11 and 15 are wrapped therearound continuously until a compact roll is produced, comprising the condenser 10 shown in Fig. 1, wherein the foil comprising the electrodes and the paper sheets comprising the 70 dielectric are in alternate relation throughout the thickness of the condenser, and the leads 11 and 15 project a considerable distance beyond one edge of the condenser in the conventional manner (not shown).

Although the sheets 14 and 17 of the dielectric are usually of a type especially selected for use in condensers, they are, like ordinary paper, readily absorbent of moisture from the atmosphere, being made up 75 essentially of cellulose particles joined together in a matrix with many very small pockets or capillary openings intricately interlaced throughout. For convenience, only one typical capillary 19 has been shown in 80 the drawing. The absorbed moisture may be held in the capillary openings 19, as water 20, (Fig. 2) and on surfaces of the particles themselves—perhaps in some cases, small amounts of the remaining salts also retain 85 a share of the moisture and complicate the conductance phenomena produced under service conditions. Some of these salts ionize, greatly decreasing the resistance of 90 the dielectric and under proper conditions 95 100

collect near the electrodes and in contact with the dielectric, causing local heating which eventually may tend toward the deterioration and breakdown of the dielectric. This normal moisture content forms conductance paths through the paper and must be removed in order to enable the condenser to function efficiently, since it is generally understood that the efficiency of a condenser in service varies inversely with the quantity of moisture contained therein. Since some of this moisture is contained as highly dispersed water in the recesses of the capillaries 19 of the dielectric, it is extremely difficult to 15 remove it therefrom by ordinary methods of evaporation. However, the importance of removing it, and the results in the way of greatly increased resistance in the dielectric to be secured by its removal, are indicated 20 by the fact that the average resistance of many typical condensers produced heretofore has been several thousand megohms less than the probable specific resistance of thoroughly dry paper dielectric. 25 This desired total drying of the dielectric may be accomplished by subjecting the dielectric to a series of three steps of treatment. Since the final step of the series will be shown hereinafter to be all-effective and 30 conclusive, under certain conditions the two preliminary steps may be dispensed with. However, since under ordinary conditions the use of all three steps affords a substantial economy of time and expense, it is preferable that they all be employed substantially as described herein.

The following description will inform as to how the invention may be practiced; however, it should be understood that it is purely 40 illustrative in purpose and is not intended to limit the invention to the specific matter disclosed therein. In a specific instance, a number of wound condensers were placed in an air-tight oven under an absolute pressure 45 of about 5 millimeters of mercury, and subjected to a temperature of 120° centigrade for 2 hours. This resulted in the evaporation of a large portion of the free or surface moisture from the dielectric, giving the condition indicated in Fig. 2, wherein it will be 50 observed that the only free moisture remaining is contained in the mouth of the capillary 19. Subsequently, a current of dry air was permitted to flow through the oven and 55 about the condensers, and the temperature of the interior of the oven maintained at approximately 120° centigrade, for approximately 2 hours. At the expiration of such 60 period all of the moisture was evaporated from the surfaces of the dielectric and a portion of the water 20 from the mouth of the capillary openings, and a condition corresponding to that indicated in Fig. 3 was produced, wherein it will be noticed that the 65 only water remaining is contained in the re-

cesses of the capillary as residual moisture.

The combined effect of the two heat treatments just described was to reduce the moisture content of the dielectric to less than one percent of its original value; but even that small amount if allowed to remain might contribute greatly to the early breakdown of the dielectric and other undesirable properties thereof, and must be removed in order to produce a dielectric of extraordinary 75 quality.

These condensers were tested immediately upon completion of these two steps and were found to possess an average resistance value of approximately 1800 megohms, but this condition will obtain for only a short while, because the application of a high potential across the dielectric, as when the condenser is in service, will cause a gradual readjustment of the moisture in the capillaries 80 and the migration of some of the water molecules outwardly to the openings of the capillaries, where they will soon contact with the electrodes and greatly reduce the resistance of the dielectric by re-establishing conductance paths therethrough.

The third step of the process was carried out by connecting a group of nine condensers 10, 10 (Fig. 5) arranged in parallel with each other, to a generator or other suitable 85 source of unidirectional current 21. A circuit for supplying the unidirectional current to the group of condensers 10, 10 included a conductor 23 extending from a switch 24 to the source 21. The switch 24 100 was connected to the conductor 23 for the purpose of opening and closing the circuit at will. A second conductor 25 connected the condensers 10 to the switch 24, and a milliammeter 26 was connected in turn to the condensers by a conductor 27. The circuit also included a field rheostat or other voltage adjuster 30 which was connected to the milliammeter 26 by a conductor 31, and a voltmeter 32 connected across the conductors 23 105 and 31.

In practice, the field rheostat 30 was adjusted to give a proper voltage and this voltage was applied across the dielectrics of the condensers by the closing of the switch 115 24. When the voltage was applied a current flowed through the dielectric and was measured by the milliammeter 26. Due to the electric charges and specific inductive capacities of both the water, and the walls of the capillary, the water 20 moved in the capillary 19 in a definite direction. This movement of the water, which exemplified the well known phenomena of electroendosmosis, caused the water to collect in particles or globules at the surface of the dielectric or in the mouth of the capillary, and the condition indicated in Fig. 4 was produced, 125 wherein it will be noted the residual water 130

20 has been entirely expelled from the recesses of the capillary.

It will be understood that the operations just described took place while the condensers were in the atmosphere used in the second heating step. Consequently, as the moisture reached the surface of the dielectric, it was vaporized by contact with the adjacent hot tin foil electrodes or evaporated into the current of dry air. After the expiration of fifteen minutes from the time of application of the initial voltage and at recurrent intervals of fifteen minutes, the voltage was successively increased by 45 volts until at the end of three hours the expulsion of the final vestiges of water from the smallest and most remote capillaries was accomplished under an applied potential of approximately 450 volts.

Since the application of too much current is apt to cause a breakdown of the dielectric, the milliammeter 26 was provided for the guidance of the operator. Although in the early stages of this third step of the process it is possible that the current might become excessive, the relative values of the potential and the resistances of the dielectric used in the condensers employed in the experiment were such as to prevent the development of too much current. For instance, in the arrangement shown in Fig. 5 of the drawing, when the nine condensers were connected in parallel and subjected to the initial potential, the current in the first instance was found to be 120 milliamperes, and this dropped sharply to 20 milliamperes, in a short time. From thence through the series of additional increases of voltages the current value varied slightly, with however a pronounced downward trend until, upon the expiration of three hours and under an applied potential of 450 volts, the current value was approximately 1/40 milliamperes. It will thus be seen that the greatest current value, namely 120 milliamperes, was reached at the first stage or concurrent with the application of the voltage; however, this amount of current is not excessive for the paper dielectrics employed, since they were subjected to it without deleterious effects.

Since the different dielectric materials and the different grades of the same material are known to possess more or less widely varying electrical characteristics, and since the current which will flow through the dielectric under a given impressed voltage will vary with the specific resistance of the particular grade of material used, and with other related electrical characteristics thereof, it is difficult, if not impossible, to determine that maximum current value which may safely be permitted to flow through a particular type of dielectric without causing dielectric breakdown, without experimenting with each type of dielectric employed. For the same reason, although it has been necessary above to des-

ignate that certain voltages were employed and for specific periods of time, and that such voltages were increased at a specified rate, it should be understood that the values used pertain necessarily only to the specific type of dielectric used, and obviously may vary in a degree to be determined by experiment where other materials are concerned.

The invention is obviously capable of successful application to other types of paper and to all materials such as absorb or retain moisture in their capillaries. It is to be understood therefore that the invention should be limited only by the scope of the appended claims.

What is claimed is:

1. A method of treating a condenser which consists of evaporating the free moisture from the dielectric thereof and expelling the residual moisture from the dielectric by electroendosmosis. 85

2. A method of treating a condenser which consists of evaporating the free moisture from the dielectric thereof, expelling the residual moisture from the dielectric by electroendosmosis and evaporating the expelled moisture. 90

3. A method of treating a condenser which consists of subjecting the dielectric material of the condenser to heat to remove the free moisture therefrom and then removing the residual moisture by applying a direct current potential across the dielectric material to produce electroendosmosis therein. 95

4. The method of manufacturing electrostatic condensers composed of paper and metallic foils formed in a roll, which consists in subjecting the condenser to a preliminary drying process and thereafter connecting the metal foils with a source of direct current potential to produce electroendosmosis in the paper and remove the residual moisture therefrom. 100

5. A method of manufacturing electrostatic condensers composed of paper and metallic foils formed in a roll, which consists in subjecting said condenser to a preliminary drying process, and thereafter connecting said metal foils with a source of current, the potential of which is successively increased to produce electroendosmosis in the paper and remove residual moisture from the paper. 110

In witness whereof, I hereunto subscribe my name this 14 day of September A. D., 1929.

RAYMOND H. HOBROCK.